

Nov. 26, 1946.

R. B. COLLINS ET AL  
PHOTOGRAPHIC MATERIAL

2,411,507

Filed Dec. 6, 1944



*Fig. 1*



*Fig. 2*



*Fig. 3*



*Fig. 4*



*Fig. 5*



*Fig. 6*

*Roland Bernard Collins* INVENTORS  
*John Miller*

BY

*Lynn Barratt Morris*  
ATTORNEY

## UNITED STATES PATENT OFFICE

2,411,507

## PHOTOGRAPHIC MATERIAL

Ronald Bernard Collins, Ilford, and John Miller,  
Nottingham, England, assignors to Ilford Limited,  
Ilford, England, a British company

Application December 6, 1944, Serial No. 566,823  
In Great Britain December 20, 1943

12 Claims. (Cl. 95-7)

1

This invention relates to photographic materials and particularly to the manufacture of dye-sensitised photographic silver halide emulsions.

Photographic silver halide emulsions have a certain natural sensitivity to light, but this is restricted to a short range of wavelengths in the ultra-violet and/or blue regions of the spectrum. The effect of incorporating a sensitising dye is to impart to the emulsion sensitivity to light of other wavelengths. It has been known for some time that the effect of incorporating in the emulsion, together with a sensitising dye, a second substance (which may or may not itself be a sensitiser) sometimes imparts an additional sensitivity to the emulsion beyond that which can be regarded as the simple additive effect of the separate substances. Combinations of sensitising dye and another substance which give this latter result are known as supersensitising combinations.

The present invention is concerned with supersensitising combinations. According to the invention, photographic silver halide emulsions are supersensitised by incorporating in the emulsion a combination of a sensitising dyestuff of the general Formula I:



where  $\text{R}_1$  and  $\text{R}_2$  are the same or different and are alkyl or aralkyl groups or substituted groups of this type,  $\text{R}_3$  is hydrogen or an alkyl or aralkyl group, and  $\text{D}_1$  and  $\text{D}_2$  are the same or different and are residues of heterocyclic nitrogen nuclei of the classes common in cyanine dyes,  $\text{A}$  is an acid radicle, and  $n$  is nought or one, and a compound of the general Formula II:



where  $\text{D}_3$  is the residue of a heterocyclic nitrogen ring (which may be the same or different from  $\text{D}_1$  or  $\text{D}_2$ ),  $\text{R}_4$  is an alkyl, aralkyl or substituted group of this type,  $\text{X}$  is a carboxyl, carboxylic ester, acyl or nitrile group, and  $\text{Y}$  is a carboxyl, carboxylic ester, nitrile or acrylic ester group, or  $\text{X}$  and  $\text{Y}$  together form the residue of a 5-membered keto-methylene ring, and  $n$  is nought or one.

The above terms, as used in the present specification and claims, have the following meaning:

Carboxyl means  $-\text{COOH}$   
Carboxylic ester means  $-\text{COOR}$   
Acyl means  $-\text{C}-\text{R}$

Nitrile means  $-\text{C}\equiv\text{N}$

Acrylic ester,  $-\text{CH}=\text{CH}-\text{COOR}$

where  $\text{R}$  is a hydrocarbon radical.

The groups  $\text{R}_1$ ,  $\text{R}_2$  and  $\text{R}_4$  are preferably lower alkyl radicles, i. e. radicles containing not more than 4 carbon atoms, e. g. methyl or ethyl, or hydroxy lower-alkyl radicles, and the group  $\text{R}_3$ , when not hydrogen, is also preferably a lower alkyl radicle, e. g. methyl or ethyl. These groups may, however, be higher alkyl radicles, or may be aralkyl radicles such as benzyl or naphthylmethyl.

10 The residues  $\text{D}_1$ ,  $\text{D}_2$  and  $\text{D}_3$  may be selected from the residues of thiazoles, oxazoles, selenazoles and their polycyclic homologues such as those of the benzene, naphthalene, acenaphthene and anthracene series, pyridine and its polycyclic homologues, such as quinoline and  $\alpha$ - and  $\beta$ -naphthaquinolines, lepidines, indolenines, diazines, such as pyrimidines and quinazolines, diazoles (e. g. thio- $\beta,\beta'$ -diazole), oxazolines, thiazolines and selenazolines. The polycyclic compounds of these series may also be substituted in the carbocyclic rings with one or more groups, such as alkyl, aryl, amino, hydroxy, alkoxy and methylene-dioxy groups, or by halogen atoms.

15 The acid radicle  $\text{A}$  may be, for example, chloride, bromide, iodide, alkyl sulphate, alkyl-p-toluene sulphonate or perchlorate.

20 In the case of the compound of general Formula II, the groups  $\text{X}$  and  $\text{Y}$ , where ester groups, are preferably lower alkyl esters. Where the group  $\text{X}$  is alkyl, aryl or aralkyl it may be, for example, methyl, ethyl or a higher alkyl group, benzyl, naphthyl-methyl, phenyl or naphthyl. Where it is an acyl group it is preferably a residue of a lower fatty acid, e. g. acetic or propionic acid. Where  $\text{X}$  and  $\text{Y}$  together form the residue of a 5-membered keto-methylene ring this may be, for example, a pyrazolone, thiopyrazolone, rhodanine, indandione or hydantoin nucleus.

25 The following are examples of specific compounds which may be employed according to this invention, the compounds being lettered to facilitate subsequent reference:

## Dyestuffs of general Formula I

- 30 A. 3,3'-diethyl-9-methyl-4.5:4'.5'-dibenzthiacarbocyanine iodide.  
B. 3,3'-triethyl-5.5'-dichloro-thiacarbocyanine chloride.  
35 C. 3,3'-diethyl-9-methyl-thiacarbocyanine bromide.  
D. 3,3'.9-triethyl-4.5:4'.5' - dibenzthiacarbocyanine iodide.  
E. 3,3'.9-triethyl-oxacarbocyanine iodide.  
40 F. 3,3'-dimethyl-9-ethyl-4.4'-dichlor-thiacarbocyanine iodide.  
G. 3,9-diethyl-3'-methyl - 4.4' - dichlor-thiacarbocyanine iodide.  
H. 3,3'-diethyl-9-methyl - 4.4' - dichlor-thiacarbocyanine iodide.

- I. 3,3'-diethyl-9,4,4'-trimethyl-thiacarbocyanine iodide.  
 J. 3,3'-4,4'-tetramethyl-9-ethyl-thiacarbocyanine iodide.  
 K. 3,3'-diethyl-9-methyl-5,6,5',6'-bis-dioxymethylene-thiacarbocyanine iodide.  
 L. 3,3'-diethyl-9-methyl-5,6,5',6'-tetramethoxy-thiacarbocyanine iodide.  
 M. 3,3'-diethyl-9-methyl-selenacarbocyanine iodide.  
 N. 3,3'-dimethyl-9-ethyl-selenacarbocyanine iodide.  
 O. 1,3'-dimethyl-10-ethyl-2-quinothiacarbocyanine iodide.

*Compounds of general Formula II*

15

- P. Ethyl-3-methyl-dihydrobenzthiazolyl-2-cyanacetate having the formula:



- Q. 3-methyl-dihydrobenzthiazolyl-2-aceto acetic ester having the formula:



- R. 3-ethyl-dihydrobenzthiazolyl-2-ethyl cyanacetate having the formula:



- S. 3-methyl-dihydro-benzoxazolyl-2-ethyl cyanacetate having the formula:



- T. 3-methyl-4:5-benzbenzthiazole-2-ethyl cyanacetate having the formula:



- V. 3-methyl-dihydrobenzthiazolyl-2-malonic ethyl ester having the formula:



- W. 4,2'(3' methyl-dihydrobenzthiazolyl)-1-phenyl-3-methyl-5-pyrazolone having the formula:



- X. 2,2'-(3' methyl-dihydrobenzthiazolyl) 1,3-indandione having the formula:



- Y. 3-methyl-dihydrobenzthiazolyl-2-acetone di-carboxylate having the formula:



- Z. 3-methyl-5,6-dimethoxy dihydrobenzthiazolyl-2-cyanacetic ethyl ester having the formula:



- ZA. 3-methyl-dihydrobenzthiazolyl-2-glutaconic diethyl ester having the formula:



- ZB. 2-dicyanethylene-3-methyl-dihydrobenzthiazole having the formula:



- ZC. 3-methyl-dihydrobenzselenaazolyl-2-ethyl cyanacetate having the formula:



- ZD. 1-ethyl-dihydroquinolylidene-2-malonic ethyl ester having the formula:



The optimum quantity of the dyestuff of general Formula I to be incorporated in the emulsion will generally be of the order of 5 to 50 cc. of a. 75 1 in 2000 solution of the dyestuff per litre of

5

emulsion. The optimum quantity of the compound of general Formula II will generally fall within the same range, but in many cases optimum results are obtained where the quantity of such compound is somewhat greater than the quantity of dyestuff used. 5

quantity of dyestuff used.

The following examples illustrate the invention. In these examples the emulsions containing the dyestuff of general Formula I and compound of general Formula II were tested for speed to daylight and to "red" light. This latter figure was obtained by exposing the emulsions to white light passing through a filter which cuts off all radiation of wavelengths less than 600 m. $\mu$ . The increase in the "red speed" shown by the supersensitised emulsions in comparison with emulsions containing only the dyestuffs of general Formula I affords a measure of the supersensitising effect obtained.

### Examples

In these examples the compounds of Formulae I and II are referred to by the letters given to them above.

The combinations of dyestuff and supersensitising compound were incorporated in a gelatin silver iodobromide emulsion containing about 6.5 gms. of silver halide (calculated as silver) per litre of emulsion, during the manufacture of the emulsion, and the resulting emulsion was coated on glass and the speed values referred to above were determined. The results are set out in the following table:

| Ex-<br>ample<br>No. | Dyestuff<br>of For-<br>mula I | Quantity<br>of dye of<br>Formula I<br>in ccs. of<br>1 in 2000<br>solution<br>per litre of<br>emulsion | Com-<br>ound<br>of<br>Formula<br>II | Quantity of<br>compound of<br>Formula I<br>in 1 ccs. of<br>1 in 1000<br>solution<br>per litre of<br>emulsion | Day-<br>light<br>speed | Red<br>speed |
|---------------------|-------------------------------|-------------------------------------------------------------------------------------------------------|-------------------------------------|--------------------------------------------------------------------------------------------------------------|------------------------|--------------|
| 1a                  | A                             | 15                                                                                                    | None                                | 7                                                                                                            | 92                     | 15           |
| 1b                  | A                             | 15                                                                                                    | P                                   | 7                                                                                                            | 107                    | 23           |
| 1c                  | A                             | 15                                                                                                    | Q                                   | 28                                                                                                           | 105                    | 24           |
| 2a                  | A                             | 22                                                                                                    | None                                | 15                                                                                                           | 145                    | 38           |
| 2b                  | A                             | 22                                                                                                    | T                                   | 15                                                                                                           | 170                    | 60           |
| 3a                  | B                             | 22                                                                                                    | None                                | 30                                                                                                           | 135                    | 50           |
| 3b                  | B                             | 22                                                                                                    | P                                   | 30                                                                                                           | 165                    | 78           |
| 4a                  | B                             | 22                                                                                                    | None                                | 32                                                                                                           | 145                    | 50           |
| 4b                  | B                             | 22                                                                                                    | R                                   | 32                                                                                                           | 180                    | 60           |
| 4c                  | B                             | 22                                                                                                    | S                                   | 4                                                                                                            | 145                    | 55           |
| 4d                  | B                             | 22                                                                                                    | T                                   | 32                                                                                                           | 160                    | 58           |
| 5a                  | C                             | 22                                                                                                    | None                                | 14                                                                                                           | 135                    | 15           |
| 5b                  | C                             | 22                                                                                                    | P                                   | 14                                                                                                           | 155                    | 19           |
| 6a                  | D                             | 22                                                                                                    | None                                | 55                                                                                                           | 134                    | 49           |
| 6b                  | D                             | 22                                                                                                    | P                                   | 55                                                                                                           | 155                    | 80           |
| 7a                  | E                             | 22                                                                                                    | None                                | 28                                                                                                           | 110                    | 11           |
| 7b                  | E                             | 22                                                                                                    | P                                   | 28                                                                                                           | 135                    | 19           |
| 8a                  | K                             | 15                                                                                                    | None                                | 30                                                                                                           | 120                    | 17           |
| 8b                  | K                             | 15                                                                                                    | P                                   | 30                                                                                                           | 330                    | 160          |
| 9a                  | K                             | 15                                                                                                    | None                                | 45                                                                                                           | 65                     | 6            |
| 9b                  | K                             | 15                                                                                                    | Z                                   | 30                                                                                                           | 93                     | 65           |

The speed values given in the foregoing table are substantially linearly related, i. e. are in direct proportion. It will be apparent from the data given in the foregoing table that the supersensitising combinations of this invention in many cases not only impart an increased sensitivity to the emulsion in the sensitising region of the dyestuff of Formula I, but actually effect an increase in the overall sensitivity of the emulsion as shown by the generally increased daylight speed. Moreover, the inclusion of the compounds of Formula II frequently produces a marked change in the distribution of the spectral sensitivity of the emulsion. These effects are illustrated by the accompanying drawing which shows spectral sensitivity curves for the emulsions of certain of the foregoing examples.

In the drawing Fig. 1 shows the spectral sensitivity curve of the emulsions of Examples 1a (full

line) and 1b (dotted line). Fig. 2 shows the spectral sensitivity curve of the emulsion of Examples 3a (full line) and 3b (dotted line). Fig. 3 shows the spectral sensitivity curve of the emulsion of Examples 6a (full line) and 6b (dotted line). Fig. 4 shows the spectral sensitivity curve of the emulsion of Examples 7a (full line) and 7b (dotted line). Fig. 5 shows the spectral sensitivity curve of the emulsion of Examples 8a (full line) and 8b (dotted line). Fig. 6 shows the spectral sensitivity curve of the emulsion of Examples 9a (full line) and 9b (dotted line).

While this invention is of particular value in connection with the supersensitizing of silver halide emulsions in gelatin, other binding colloids for the emulsion may be employed, for example polyvinyl alcohol, polyvinyl acetals, partially hydrolysed cellulose esters and the like.

What we claim is:

What we claim is:

1. Silver halide photographic emulsions containing a sensitizing dyestuff of the general formula:



where  $R_1$  and  $R_2$  are each selected from the group consisting of alkyl and aralkyl groups,  $R_3$  is selected from the group consisting of the hydrogen atom, alkyl and aralkyl groups,  $D_1$  and  $D_2$  are each selected from the group consisting of residues of heterocyclic nitrogen nuclei,  $A$  is an acid radicle and  $n$  is selected from the group consisting of nought and one, and a compound of the general formula:



where  $D_3$  is selected from the same class as  $D_1$  and  $D_2$ ,  $R_4$  is selected from the same class as  $R_1$  and  $R_2$ ,  $X$  is selected from the class consisting of the carboxyl, carboxylic ester, acyl and nitrile groups, and atoms which with  $Y$  form the residue of a 5-membered keto-methylene ring, and  $Y$  is selected from the group consisting of carboxyl, carboxylic ester, nitrile and acrylic ester groups and atoms which with  $X$  form the residue of a 5-membered keto-methylene ring, and  $n$  is selected from the group consisting of nought and one.

2. Silver halide photographic emulsions containing a sensitizing dyestuff of the general formula:



60 where  $R_1$  and  $R_2$  are each selected from the group consisting of alkyl and aralkyl groups,  $R_3$  is selected from the group consisting of the hydrogen atom, alkyl and aralkyl groups,  $D_1$  and  $D_2$  are each the residues of azole nuclei,  $A$  is an acid radicle and  $n$  is selected from the group consisting of nought and one, and a compound of the general formula:

65



where  $D_3$  is selected from the same class as  $D_1$  75 and  $D_2$ ,  $R_4$  is selected from the same class as

$R_1$  and  $R_2$ ,  $X$  is selected from the class consisting of the carboxyl, carboxylic ester, acyl and nitrile groups and atoms which with  $Y$  form the residue of a 5-membered keto-methylene ring, and  $Y$  is selected from the group consisting of carboxyl, carboxylic ester, nitrile and acrylic ester groups and atoms which with  $X$  form the residue of a 5-membered keto-methylene ring, and  $n$  is selected from the group consisting of nought and one.

3. Silver halide photographic emulsions containing a sensitizing dyestuff of the general formula:



where  $R_1$  and  $R_2$  are each selected from the group consisting of alkyl and aralkyl groups,  $R_3$  is selected from the group consisting of the hydrogen atom, alkyl and aralkyl groups,  $D_1$  and  $D_2$  are each selected from the group consisting of residues of heterocyclic nitrogen nuclei,  $A$  is an acid radicle and  $n$  is selected from the group consisting of nought and one, and a compound of the general formula:



where  $D_3$  is a residue of an azole nucleus,  $R_4$  is selected from the same class as  $R_1$  and  $R_2$ ,  $X$  is selected from the class consisting of the carboxyl, carboxylic ester, acyl and nitrile groups and atoms which with  $Y$  form the residue of a 5-membered keto-methylene ring, and  $Y$  is selected from the group consisting of carboxyl, carboxylic ester, nitrile and acrylic ester groups and atoms which with  $X$  form the residue of a 5-membered keto-methylene ring, and  $n$  is selected from the group consisting of nought and one.

4. Silver halide photographic emulsions containing a sensitising dyestuff of the general formula:



where  $R_1$  and  $R_2$  are each selected from the group consisting of alkyl and aralkyl groups,  $R_3$  is selected from the group consisting of the hydrogen atom, alkyl and aralkyl groups,  $D_1$  and  $D_2$  are each the residues of azole nuclei,  $A$  is an acid radicle and  $n$  is selected from the group consisting of nought and one, and a compound of the general formula:



where  $D_3$  is a residue of an azole nucleus,  $R_4$  is selected from the same class as  $R_1$  and  $R_2$ ,  $X$  is selected from the class consisting of the carboxyl, carboxylic ester, acyl and nitrile groups and atoms which with  $Y$  form the residue of a 5-membered keto-methylene ring, and  $Y$  is selected from the group consisting of carboxyl, carboxylic ester, nitrile and acrylic ester groups and atoms which with  $X$  form the residue of a 5-membered keto-methylene ring, and  $n$  is selected from the group consisting of nought and one.

5. Silver halide photographic emulsions con-

taining a sensitising dyestuff which is a compound of the general formula:



10 where  $R_1$  and  $R_2$  are each selected from the group consisting of alkyl and aralkyl groups,  $R_3$  is selected from the group consisting of the hydrogen atom and alkyl and aralkyl groups,  $M_1$  and  $M_2$  are each the residue of a thiazole nucleus and  $A$  is an acid radicle, and a compound of the general formula:



where  $M_3$  is a residue of a thiazole nucleus,  $R_4$  is selected from the same class as  $R_1$  and  $R_2$ ,  $X$  is selected from the class consisting of the carboxyl, carboxylic ester, acyl and nitrile groups and atoms which with  $Y$  form the residue of a 5-membered keto-methylene ring, and  $Y$  is selected from the group consisting of carboxyl, carboxylic ester, nitrile and acrylic ester groups and atoms which with  $X$  form the residue of a 5-membered keto-methylene ring.

6. Silver halide photographic emulsions containing a sensitising dyestuff which is a compound of the general formula:



where  $R_1$  and  $R_2$  are each selected from the group consisting of alkyl and aralkyl groups,  $R_3$  is selected from the group consisting of the hydrogen atom and alkyl and aralkyl groups,  $M_1$  and  $M_2$  are each the residue of a benzthiazole nucleus and  $A$  is an acid radicle, and a compound of the general formula:



55 where  $M_3$  is a residue of a benzthiazole nucleus,  $R_4$  is selected from the same class as  $R_1$  and  $R_2$ ,  $X$  is selected from the class consisting of the carboxyl, carboxylic ester, acyl and nitrile groups and atoms which with  $Y$  form the residue of a 5-membered keto-methylene ring, and  $Y$  is selected from the group consisting of carboxyl, carboxylic ester, nitrile and acrylic ester groups and atoms which with  $X$  form the residue of a 5-membered keto-methylene ring.

60 7. Silver halide photographic emulsions containing a sensitising dyestuff which is a compound of the general formula:



where  $R_1$  and  $R_2$  are each lower alkyl groups,  $R_3$  is a lower alkyl group,  $M_1$  and  $M_2$  are each the

9

residue of a thiazole nucleus and A is an acid radicle, and a compound of the general formula:



where  $M_3$  is a residue of a thiazole nucleus,  $R_4$  is a lower alkyl group,  $X$  is selected from the class consisting of the carboxyl, carboxylic ester, acyl and nitrile groups and atoms which with  $Y$  form the residue of a 5-membered keto-methylene ring, and  $Y$  is selected from the group consisting of carboxyl, carboxylic ester, nitrile and acrylic ester groups and atoms which with  $X$  form the residue of a 5-membered keto-methylene ring.

8. Silver halide photographic emulsions containing a sensitising dyestuff which is a compound of the general formula:



where  $R_1$  and  $R_2$  are each lower alkyl groups,  $R_3$  is a lower alkyl group,  $M_1$  and  $M_2$  are each the residue of a benzthiazole nucleus and A is an acid radicle, and a compound of the general formula:



where  $M_3$  is a residue of a benzthiazole nucleus,  $R_4$  is a lower alkyl group,  $X$  is selected from the class consisting of the carboxyl, carboxylic ester, acyl and nitrile groups and atoms which with  $Y$  form the residue of a 5-membered keto-methylene ring, and  $Y$  is selected from the group consisting of carboxyl, carboxylic ester, nitrile and acrylic ester groups and atoms which with  $X$  form the residue of a 5-membered keto-methylene ring.

9. Silver halide photographic emulsions containing a sensitising dyestuff which is a compound of the general formula:



where  $R_1$  and  $R_2$  are each lower alkyl groups,  $R_3$  is a lower alkyl group,  $M_1$  and  $M_2$  are each the residue of a thiazole nucleus and A is an acid radicle, and a compound of the general formula:



where  $M_3$  is a residue of a thiazole nucleus,  $R_4$  is a lower alkyl group,  $X$  is a carboxylic ester group, and  $Y$  is selected from the group consisting of carboxyl, carboxylic ester, nitrile and acrylic ester groups and atoms which with  $X$  form the residue of a 5-membered keto-methylene ring.

10

10. Silver halide photographic emulsions containing a sensitising dyestuff which is a compound of the general formula:



where  $R_1$  and  $R_2$  are each lower alkyl groups,  $R_3$  is a lower alkyl group,  $M_1$  and  $M_2$  are each the residue of a thiazole nucleus and A is an acid radicle, and a compound of the general formula:



where  $M_3$  is a residue of a thiazole nucleus,  $R_4$  is a lower alkyl group,  $X$  is a carboxylic ester group, and  $Y$  is a nitrile group.

11. Silver halide photographic emulsions containing a sensitising dyestuff which is a compound of the general formula:



where  $R_1$  and  $R_2$  are each lower alkyl groups,  $R_3$  is a lower alkyl group,  $M_1$  and  $M_2$  are each the residue of a benzthiazole nucleus and A is an acid radicle, and a compound of the general formula:



where  $M_3$  is a residue of a benzthiazole nucleus,  $R_4$  is a lower alkyl group,  $X$  is a carboxylic ester group, and  $Y$  is selected from the group consisting of carboxyl, carboxylic ester, nitrile and acrylic ester groups and atoms which with  $X$  form the residue of a 5-membered keto-methylene ring.

12. Silver halide photographic emulsions containing a sensitising dyestuff which is a compound of the general formula:



where  $R_1$  and  $R_2$  are each lower alkyl groups,  $R_3$  is a lower alkyl group,  $M_1$  and  $M_2$  are each the residue of a benzthiazole nucleus and A is an acid radicle, and a compound of the general formula:



where  $M_3$  is a residue of a benzthiazole nucleus,  $R_4$  is a lower alkyl group,  $X$  is a carboxylic ester group, and  $Y$  is a nitrile group.

RONALD BERNARD COLLINS.  
JOHN MILLER.